

# United States Patent [19]

Kennedy

[11] 3,844,964

[45] Oct. 29, 1974

[54] EXTREME PRESSURE LUBRICATING OIL ADDITIVE

|           |         |                |            |
|-----------|---------|----------------|------------|
| 2,370,756 | 3/1945  | Sibley .....   | 252/48.2 X |
| 3,114,713 | 12/1963 | Coffield ..... | 252/48.2   |
| 3,442,806 | 5/1969  | O'Neill.....   | 252/48.2 X |

[75] Inventor: Brian R. Kennedy, San Rafael, Calif.

[73] Assignee: Chevron Research Company, San Francisco, Calif.

[22] Filed: Nov. 20, 1972

[21] Appl. No.: 308,227

[52] U.S. Cl..... 252/48.2, 260/609 F

[51] Int. Cl..... C10m 1/42

[58] Field of Search ..... 252/48.2, 609 F

## [56] References Cited

### UNITED STATES PATENTS

2,253,228 8/1941 Cantrell et al. .... 252/48.2 X

*Primary Examiner*—W. Cannon

*Attorney, Agent, or Firm*—G. F. Magdeburger; C. J. Tonkin; S. R. La Paglia

[57]

## ABSTRACT

A thio bis(dialkylphenol), wherein the alkyl substituents are C<sub>1</sub>-C<sub>20</sub> groups with the proviso that the total number of substituent carbon atoms is at least 10, is found to be a superior extreme pressure additive.

2 Claims, No Drawings

## EXTREME PRESSURE LUBRICATING OIL ADDITIVE

## BACKGROUND OF THE INVENTION

## 1. Field of the Invention

A lubricating oil performs several functions related to the lubrication of metallic surfaces which requires the oil to act as a carrier of functional additives such as dispersants, detergents, extreme pressure agents, viscosity index improvers, etc. There are few commercial examples of an ashless extreme pressure agent. Such an additive is of importance in formulating industrial greases and oils for internal combustion engines operating on unleaded fuels. The purpose of this work was to develop such an ashless additive. Extreme pressure agents also find use in functional fluids and fuels. Dialkyl-substituted phenols wherein the alkyl must be branched at the alpha-carbon atom (so-called "hindered" phenols) and wherein the thio bridge is para, e.g., 4,4'-thio-bis(2,6-ditert-butylphenol), are known in the prior art as antioxidant additives. U.S. Pat. Nos. 3,326,800 and 3,250,712.

## SUMMARY OF THE INVENTION

A thio bis(dialkylphenol), which is preferably mono- or dithio ortho-bridged and in which the alkyl groups are C<sub>1</sub>-C<sub>20</sub> with the proviso that the total number of substituent carbon atoms is at least 10, functions as a superior extreme pressure additive. The additive is, for example, the reaction product of an alkylated cresol, preferably an o-cresol, with sulfur monochloride.

## DETAILED DESCRIPTION OF THE INVENTION

Lubricating oil, fuel and functional fluid additives which function as extreme pressure agents are prepared from the reaction of a dialkylated phenol with sulfur monochloride.

It is an essential feature of the invention that the phenol be di-substituted with C<sub>1</sub>-C<sub>20</sub> alkyl groups, such that the total number of carbons substituted on the phenol is at least 10. It is preferred that one of the alkyl groups is ortho to the phenolic hydroxy group and the other alkyl is para. The presence of ortho alkyl substituents, or ortho-para substituents reduces the probability of other than the ortho-bridged bis structures in the sulfurized product.

The sulfurization is preferably performed with sulfur monochloride, S<sub>2</sub>Cl<sub>2</sub>, but other sulfurizing agents may be utilized. The product has a structural formula:



wherein R and R' are the C<sub>1</sub>-C<sub>20</sub> alkyl groups previously described and may be the same or different.

Examples of such alkyl groups include methyl, ethyl, dodecyl, isopropyl, n-butyl, s-butyl, tert.butyl, hexyl, 2-methylhexyl and less than C<sub>20</sub> oligomers of C<sub>2</sub>-C<sub>5</sub> monomeric mono-olefins such as tetrapropenyl or di-butyl.

Examples of such dialkylated phenols include methyl nonyl phenol, methyl dodecyl phenol, dipentyl phenol, ethyl undecyl phenol, propyl decyl phenol, butyl nonyl

phenol, amyl octyl phenol, hexyl heptyl phenol, methyl polypropenyl phenol, ethyl polyisobutenyl phenol, ditetrapropenyl phenol, etc.

The value of n can be 1-4, more usually in the range of 1 to 2 and the disulfide is particularly preferred. The weight percent of sulfur is preferably within the range of from 5 to 30 percent and most preferably in the range of 5 to 10 percent.

Various methods of preparing sulfurized alkyl phenols are known in the art. The particular method employed is not critical to this invention, although some methods will be favored over others by providing higher weight percents of sulfur. U.S. Pat. No. 2,409,687 describes a method of sulfurizing using sulfur monochloride and the alkylphenol in an inert solvent. U.S. Pat. No. 2,680,096 and 3,178,368 describe sulfurizing using sulfur with calcium phenoxide in the presence of ethylene glycol.

Depending on the method of sulfurization, various solvents or dispersants may be used. Illustrative of such solvents are oil, particularly hydrocarbonaceous fluids used as lubricating oils, inert hydrocarbons, both aromatic and aliphatic, etcetera. The concentration of the reactants may be varied widely. In sulfurizing with sulfur, the weight ratio of sulfur to alkylphenol will be in the range of 1:0.9-10, usually about 1:2-6. Elevated temperatures will be used, the degree depending on the particular reactants. Generally, temperatures for sulfurization with sulfur will be in the range of about 200° to 350°F. In sulfurization with sulfur monochloride, the reaction mixture will be refluxed with stirring and the sulfurmonochloride will be slowly added as illustrated in the following examples.

Example 1: Alkylation of o-cresol with propylene tetramer

o-cresol (540 grams), propylene tetramer (840 grams), and clay catalyst (85 grams) were placed in a 2-liter flask equipped with stirrer, reflux condenser, and thermometer. The stirred mixture was heated at 150°C ± 6°C for 3 hours, cooled, and filtered. The filtrate was stripped at 110°C and 8 mm. vacuum to give tetrapropenyl o-cresol (899 grams). Hydroxyl number, 192 mg KOH/g; equivalent weight, 292; calculated for C<sub>19</sub>H<sub>32</sub>O, 276.

Example 2: Sulfurization of Tetrapropenyl o-Cresol

Tetrapropenyl o-cresol (898 grams) was taken up in n-heptane (800 ml.). To the solution was added sulfur monochloride (80.4 ml., 135 grams) with stirring during 1½ hours. The stirred solution was heated under reflux for 2 hours, cooled to 80°C, and 1,000 ml. of water was added. The heptane layer was separated, washed with water (three times at 1,000 ml.), and dried with Na<sub>2</sub>SO<sub>4</sub>. Evaporation gave the sulfurized phenol (758 grams); percent Cl, 0.67 percent by weight.

Example 3:

234 grams of substantially dipentylated phenol was diluted with n-heptane (500 ml.) and sulfurmonochloride (80.4 ml., 135 grams, about 1 mol) was added dropwise with stirring during 2 hours. The stirred solution was heated under reflux with a nitrogen purge for 2 hours, cooled, and 400 ml. of water was added. After stirring for another hour the heptane layer was separated, washed with water (10 times at 500 ml.), and dried with Na<sub>2</sub>SO<sub>4</sub>. Evaporation gave the sulfurized phenol (218 grams); percent chlorine, 0.21 percent.

Example 4: Alkylation of p-tetrapropenyl phenol with C<sub>7</sub>-C<sub>9</sub> olefin

To the mono substituted phenol (352.7 grams), and C<sub>7</sub>-C<sub>9</sub> alpha olefins (165.7 grams) was added clay catalyst (35 grams). The stirred mixture was heated under reflux at 135°C for 2 hours, cooled to 100°, and filtered. The filtrate was stripped at 120°C and 8 mm. vacuum to give the dialkylated phenol (360 grams); hydroxyl number, 139 mg KOH/g; equivalent weight, 403; calculated for C<sub>26</sub>H<sub>46</sub>O, equivalent weight, 374.

Example 5:

The dialkylated phenol product of Example 4 (358.4 grams) in 700 ml. of n-heptane was stirred with 36 ml. of sulfur monochloride added drop-wise. The solution was heated under reflux for 2 hours with a nitrogen purge. To the cooled (80°C) product was added 500 ml. of water with stirring. The heptane layer was separated, washed with water (twice at 600 ml.), and dried with Na<sub>2</sub>SO<sub>4</sub>. Evaporation gave the sulfurized phenol (369 grams); percent Cl, 0.11 percent.

The compositions of this invention can be used with a variety of greases and oils, that is, fluids of lubricating viscosity, fuels and functional fluids. Base oils include such naturally occurring oils as naphthenic base, paraffin base, asphaltic base and mixed base lubricating oils. Other lubricants include lubricating oils derived from coal products, synthetic oils such as polymers of propylene, butylene, etc., aromatic hydrocarbons, halogenated aromatic hydrocarbons, etc. Other illustrative oils are the esters of organic and inorganic acids, e.g.

shaft. The load at failure in pounds is taken as a quantitative measure of the EP property of the oil composition. Mineral oils in general will fail at 600-900 pounds. Oils with moderate EP additives will fail at 5 2,000-1,500 pounds and very effective extreme pressure additives will permit loadings in excess of 3,000 pounds. The extreme pressure properties of the additives of the present invention are illustrated and compared in the Falex test machine results given in Tables I and II.

TABLE I

|           | Additive | Conc., Wt. % | Falex Failure <sup>1</sup><br>pounds |
|-----------|----------|--------------|--------------------------------------|
|           | None     | —            | 900                                  |
| Example 5 | 1        | —            | 1300                                 |
|           | 2        | —            | 4300                                 |
| Example 2 | 1        | —            | 4500                                 |
|           | 2        | —            | 4400                                 |
| Example 3 | 1        | —            | 4500                                 |
|           | 2        | —            | 4300                                 |

<sup>1</sup>Mean value.

<sup>2</sup>A neutral paraffinic base oil of viscosity about 480 SUS at 100°F with 5 weight percent of polyisobutylene succinimide and 0.1 weight percent of terephthalic acid.

25

It is evident from Tables I and II that the thio bis(dialkylphenol) additives wherein the substituents contain a total of at least 10 carbon atoms are satisfactory 30 extreme pressure agents.

TABLE II

| Additive, Wt. % <sup>1</sup>                   | Compositions |      |      |      |      |      |      |     |
|------------------------------------------------|--------------|------|------|------|------|------|------|-----|
|                                                | 1            | 2    | 3    | 4    | 5    | 6    | 7    | 8   |
| Thio bis(monoalkylphenol) <sup>2</sup>         | 1.5          | —    | —    | —    | —    | —    | —    | —   |
| 4,4-methylene bis(2,6-di-<br>tert-butylphenol) | 1.25         | 1.25 | 1.25 | 1.25 | —    | —    | —    | —   |
| Example 2                                      | —            | —    | 1.0  | 2.0  | 1.0  | 1.5  | 2.0  | —   |
| Falex Shear                                    | 2650         | 900  | 4150 | 4250 | 4250 | 4250 | 4250 | 300 |
| Load at failure, pounds                        |              |      |      |      |      |      |      |     |

<sup>1</sup>Base oil in a neutral paraffin oil of viscosity about 480 SUS at 100°F with 6.25 weight percent of polyisobutylene succinimide, 0.1 weight percent of terephthalic acid and 1.0 weight percent of diparaffin polysulfide.

<sup>2</sup>A monotetrapropenyl phenol.

carboxylates such as octylsebacate, etc. and silicates and phosphates, alkylene oxides and polymers thereof may also be used. The base oils may be used individually or in combination, whenever miscible or made so by the use of mutual solvents. Oils of lubricating viscosity are normally defined as those having viscosities at 45 100°F in the range of 35-50,000 SUS.

The additives of this invention will generally be present in lubricating oils in amounts of from about 0.5 to 20 weight percent of the total composition, more usually in amounts of from about 1 to 4 weight percent of 55 the total composition.

Evaluation

In order to demonstrate the enhanced effectiveness of the compositions of this invention as additives in lubricating oils and greases, a number of tests were carried out to determine their effectiveness as extreme pressure agents. The additive compositions were evaluated in the Falex shear test. In the Falex test, stationary vee-blocks are pressed on either side of a rotating steel shaft by a nutcracker arrangement of lever arms. Test specimens are immersed in a tank of test lubricant which is at a known temperature. Loading is automatically increased until seizure occurs. The failure point is indicated by shearing of the pin holding the vertical

50 In addition to the additives described in this invention, the lubricating compositions may also contain other lubricating oil and grease additives such as oiliness agents, extreme pressure agents, rust inhibitors, oxidation inhibitors, corrosion inhibitors, viscosity index improving agents, dyes, detergents, dispersants, etc. Usually, for oils to be used in internal combustion engines, the amount of these additives will range from about 0.1-20 percent by weight, and more usually from about 0.5-10 weight percent. The individual additives may vary in amounts from about 0.01-10 weight percent of the total composition. In concentrates, the weight percent of these additives will usually range from about 0.3-60 weight percent.

I claim:

60 1. A lubricating composition comprising a major amount of an oil of lubricating viscosity and from 0.5 to 20 weight percent of at least one compound of the formula:



wherein R' is an alkyl group of from 10 to 20 carbon atoms and n is an integer of from 1 to 4.

2. A lubricating oil composition according to claim 1 wherein R' is dodecyl.

\* \* \* \* \*

5

10

15

20

25

30

35

40

45

50

55

60

65